# EUROPEAN PATENT SPECIFICATION

(11) **EP 1 113 085 B1**
(45) Date of publication and mention of the grant of the patent: **21.05.2003**
(21) Application number: 99870267.4
(22) Date of filing: 17.12.1999
(51) Int. Cl.: C22C 38/02, C22C 38/22

(54) **Method of production of cold-rolled metal coated steel products, and the product obtained, having a low yield ratio**
Verfahren zum Herstellen von kaltgewalzten metallbeschichteten Stahlprodukte mit niedrigem Streckgrenze-Zugfestigkeit, und dabei erhaltene Produkte
Méthode de production de produits en acier laminés à froid revêtus de métal présentant un bas rapport entre limite d'élasticité et charge à la rupture, et produits ainsi obtenus.

(43) Date of publication of application: 04.07.2001
(73) Proprietor: SIDMAR N.V., B-9042 Gent (BE)
(72) Inventor: Claessens, Serge, B-2100 (BE); Vanderschueren, Dirk, B-9820 Merelbeke (BE)
(74) Representative: Van Malderen, Joelle

(56) References cited:
- EP-A- 0 040 553
- GB-A- 1 287 178
- PATENT ABSTRACTS OF JAPAN vol. 018, no. 296 (C-1209), 6 June 1994 (1994-06-06) -& JP 06 057375 A (SUMITOMO METAL IND LTD), 1 March 1994 (1994-03-01)

## Description

### Field of the invention

The present invention is related to a method of production of a high strength cold-rolled metal coated steel product.

The present invention is also related to the direct products obtained by the method mentioned her above.

### State of the art

There is a need in the automobile field for cold-rolled hot dip coated steel products having a low yield ratio as well as a tensile strength comprised between 500 MPa and 800 MPa, likewise for steel grades with a high temperature corrosion resistance up to 900°C in combination with good mechanical properties during and after their use at these high temperatures.

Those steels are also commonly called multi-phase steels or preferably dual phase steels.

Documents US-A-4394186 and BE-A-886583 are describing dual phase steel sheets having as major constituents a phase being ferrite and at least another phase being either martensite or bainite or retained austenite. These steel sheets have a low yield ratio, of approximately 0.6, and are free from yield point elongation. The production method for obtaining uncoated steel sheets is to heat the steel in a continuous annealing line at a temperature within the intercritical region followed by a quenching in one step(called primary cooling R1) from the annealing temperature to a temperature lower than 200°C with an average cooling rate comprised between 1°C and 30°C per second. The composition of the steel has a carbon content comprised between 0.01 to 0.3% with a manganese content comprised between 0.7 and 1.7%.

The production method for obtaining a hot dip coated steel is to heat the steel in a continuous annealing line at a temperature within the intercritical region followed by a quenching in two steps: in the first quenching step, the strip is quenched (primary cooling R1) down to a temperature between 420°C and 700°C (molten zinc bath temperature) at a cooling rate comprised within the range of 1°C/sec < R1 < 30°C/sec, the second quenching step (secondary cooling R2) consists in a quenching from the molten bath temperature to a temperature lower than 200°C at a cooling rate within the range of 100°C/sec < R2 < 300°C/sec. The first quenching step is to avoid the transformation of austenite to perlite, the second quenching step is performed to obtain the transformation of the austenite into martensite. The described high (between 100°C and 300°C per second) secondary cooling rate (R2) of the steel strip which is still covered with molten metal, is probably feasible at laboratory scale, but in the industrial technology of today this quenching is not feasible. Indeed, after the molten metal coating bath the coated strip (with molten metal at its surface) is cooled in open air (no forced air cooling) during its vertical transfer to the wiping knifes (regulation of the layer thickness) and is then cooled in a vertical cooling device, to ensure the same layer thickness on both sides. A cooling rate, higher than 50°C per second can only be achieved by roll quenching, which is not applicable in said method due to the molten layer, or by water quenching, which is impossible to apply in said method on a molten metal surface and above a molten metal bath. Those two quenching methods are applied on uncoated steel surfaces. So far in the state of the art, no industrial galvanising line has been equipped with such quenching devices used for secondary quenching.

EP-A-0501605 describes a galvanised steel sheet, which has a tensile strength not less than 800Mpa and a yield ratio lower than 0.6. This steel contains carbon, manganese, niobium, titanium and boron and has a dual phase structure. After annealing at a temperature comprised between Ac3-30°C to Ac3+70°C the steel sheet is cooled at a rate higher than 50°C per second down to a temperature comprised between 450°C and 550°C. This controlled cooling step should avoid that the perlite transformation occurs. The addition of manganese and chrome as alloying elements as a way of obtaining quenching structures is well known. Those elements have however a very detrimental effect on the adhesion of the coating metal on the steel surface.

JP-A-4350152 describes the manufacture of a galvanised steel sheet having a molybdenum content comprised between 0.005 and 0.5%, a boron-content comprised between 4 and 50 ppm, a silicon-content less than 0.5% and a carbon-content comprised between 0.01 and 0.2% with the presence of some Mn, Al and Ti elements. The annealing temperature at the galvanising line lies higher than Ac3. The cooling is performed at a cooling rate higher than 50°C per second. This method has two main disadvantages: the high annealing temperature of above Ac3 is very expensive and the high cooling rate (> 50°C/second) in the secondary cooling, is hardly feasible industrially .

JP-A-56047555 is describing the manufacture of a galvanised steel plate by annealing a cold rolled steel strip through a continuous hot dip galvanising line.

The steel composition consists of 0.02-0.07% C, 1.5-2.5% Mn, 0.5-1%Cr, 0.01-0.1% Al, 0.07% or less Si, and the remaining is Fe. The Mn, Cr and C-contents are defined by the following relation:$\text{C + 0,06 Mn + 0.03 Cr > 0.17%.}$

The steel strip is soaked between the transformation temperatures Ac1 and Ac3, and soon passed through the hot galvanising bath of the said hot dip galvanising line to obtain the galvanised steel plate having a low yield ratio of approx. 0.7 or less and a tensile strength of approx. 450MPa or more. The high Mn(>1.5%) and Cr (>0.5%) concentrations have such a detrimental effect on the zinc adhesion that it is virtually impossible to obtain a defect free zinc layer for industrial applications. This is due to the heavy manganese and chrome oxides formed at the strip surface before entering the zinc bath.

JP-A-56163219 is describing a cold rolled high-tensile galvanised steel strip whereby a slab of the steel consisting of 0.02-0.15%C, 1.6-3.0% Mn, 0.1-1.0% Cr, less than 0.1% Si, 0.01-0.10% Al and the balance Fe with unavoidable impurities and satisfying the following relation : Mn%+1/2Cr% higher than or equal to 1.9%, is hot-rolled, pickled and cold-rolled to obtain a cold-rolled steel strip. Then, the slab is heated at an annealing temperature between Ac1 and Ac3 with an in-line annealing type continuous galvanising device and is immediately passed through a galvanising bath, whereby it is plated. The average cooling rates up to the execution of the hot dipping after the in-line annealing are preferably about 2-8°C/sec and the average cooling rates down to about 350 °C after the plating are preferably about 3-8 °C/sec. The high Mn (>1.5%) and Cr (>0.5%) concentrations have such a detrimental effect on the zinc adhesion that it is virtually impossible to obtain a defect free zinc layer for industrial applications. This is due to the heavy manganese and chrome oxides formed at the strip surface before entering the zinc bath.

Aluminising steel according to the above described process of annealing and cooling in two steps is also a known technique. For high temperature applications, a combination of a good adhesion of the coating, together with a low decrease in strength because of the use at high temperature is necessary. Aluminium coatings on standard commercial sheet steels show a poor temperature corrosion resistance above 650°C, because of the formation of brittle Al-Fe-Si-compounds.

By adding alloying elements like Ti in the steel, aluminised steel grades have been made commercially available in the past with a high temperature corrosion resistance up to 800°C. One commercial steel grade is known to have a good behaviour at 900°C. A weakness of those steels is the continuous decrease in strength during the use time, related to the time spent at high temperature. To thwart the decrease in strength in this existing grade considerable amounts of Ti and Nb are added to the steel in order to inhibit the ferrite grain growth. However, by doing this, the decrease in strength is only retarded.

### Aims of the invention

The present invention aims to produce a cold-rolled hot-dip metal coated multi-phase steel, having a tensile strength of at least 500 MPa, and a yield ratio (Re/Rm) lower than 0.65 in skinned condition and lower than 0.60 in unskinned condition.

The present invention aims to suggest a high strength steel with good formability and good metal coating adhesion behaviour, which are required for instance by the automobile industry for unexposed and exposed parts.

A further aim is to suggest an aluminised steel having a high temperature corrosion resistance up to 900°C, good coating adhesion and good strength properties during and after its use at these high temperatures.

### Main characteristics of the present invention

The present invention relates to a method and a composition for producing a cold-rolled steel sheet with multi-phase structure and more particularly to a method and a composition for producing a cold-rolled metal coated steel sheet having excellent formability, high strength, low yield ratio and high ductility.

More specific for the aluminised steel the present invention makes it possible to obtain an increase in strength by using it at high temperature, in combination with a good coating adhesion and a low yield ratio. Furthermore, because of the metallurgy of the steel, the mechanical values are reconditioned through its use at high temperature.

The term "multiphase" used here designates that the major constituent phases of the steel are a ferrite phase and a martensite phase. Advantageously in addition of those two phases a low amount of a bainite phase and of a retained austenite phase could be present.

The term "yield ratio" designates the ratio: yield strength/tensile strength i.e. Re/Rm.

As a first object, the present invention is more particularly related to a steel composition comprising:
- A C- content, between 0.06 weight% (hereafter denoted as %) and 0.15%,
- A Si-content, between 0.1% and 0.4%,
- A Mn-content, lower than 1.5%,
- A Cr-content, between 0.2% and 0.5%,
- A Mo-content, between 0.1% and 0.25%, so that the following condition is met: Cr + 2Mo ≥ 0.7%,
- the balance being Fe and incidental impurities.

As a second object, the invention also 5 relates to a method of producing a cold-rolled, metal coated, multi-phase steel having the above composition, said method comprising the steps of:
- preparing a steel sheet by slab reheating, hot rolling and cold rolling,
- soaking said cold-rolled steel sheet at a temperature between Ac1 and Ac3,
- performing a primary cooling down to the temperature of the molten metal bath, with a cooling rate, higher than 25°C per second,
- performing the hot dip metal coating of said steel sheet,
- performing a secondary cooling of said steel sheet to a temperature lower than Ms, with a cooling rate, higher than 4°C per second,
- performing a skin-pass reduction between 0% and 0.4%.

As a third object, the invention also relates to the end product, which is a steel product having said composition, which is produced by said method and which is characterised by :
- a tensile strength of at least 500MPa,
- a yield ratio lower than 0.65 in skinned condition and lower than 0.6 in unskinned condition.
- a superior coating adhesion.
- in the case of the aluminised steel, a temperature corrosion resistance up to a temperature of 900°C.

### Short description of the drawings

Figure 1 represents a schematic view of the annealing treatment at the hot dip coating line according to the method of the present invention. Additions of Cr and Mo retard the austenite transformation into perlite and bainite.

Figure 2 represents the influence of Cr-addition on the formation of Cr₂O₃ on the surface of the steel sheet after soaking and before hot dip coating.

Figures 3a and 3b are representing industrial trial results, for the galvanised steel product according to the present invention, wherein :
(3a) represents the obtained yield-strength (Re) and the tensile strength (Rm) respectively while
(3b) represents the obtained yield ratio (Re/Rm) as a function of the soaking temperature.

Figure 4 represents the influence of the skin-pass reduction on the yield ratio of the galvanised steel product according to the present invention.

Figure 5 represents the temperature resistance of aluminised steel according to the present invention, compared to existing steels.

Figure 6 represents the strength in terms of yield strength Re and tensile strength Rm as a function of the number of hours spent at a high temperature.

Figure 7 compares the coating quality of an aluminised steel according to the present invention to that of an existing steel, after a prolonged exposure to 800°C.

Figure 8 illustrates the ability of the aluminised steel according to the present invention to retain its mechanical properties after cooling from a high temperature (reconditioning of the steel).

### Description of preferred embodiments of the invention for the production of a hot dip metal coated sheet

The following description is related to two embodiments of the method according to the present invention, namely for the production of a preferred galvanised steel sheet and for the production of a preferred aluminised steel sheet.

For the development of a quality of steel sheets as required by the automobile industries, a compromise has to be found between the coating properties and the mechanical properties. Sufficient alloying elements need to be added to increase the quenchability, i.e. elements that prevent as much as possible the transformation of the austenite (formed at soaking temperature) into bainite before reaching the Ms (Martensite Start) temperature. The quenching effect is more difficult to obtain on a hot dip coating line due to the processing through the molten metal bath and therefore the inevitable quasi-isotherm remaining at the molten metal temperature (400°C to 700°C). This is schematically represented in Figure 1.

Elements that can theoretically be taken into account to increase the quenchability are B, C, Mo, Cr, Si, and Mn. As it has been discussed in the state of the art section, too high levels of Cr and Mn lead to a deterioration of the coating layer adhesion.

However, in the case of the aluminised steel sheet, these elements (Mn and Cr, also Ti) are essential in avoiding the formation of brittle Fe-Al-Si compounds during the use at high temperatures, which are detrimental for the coating adhesion. The presence of Mn, Cr and Ti is beneficial for the phenomenon of interdiffusion of Fe and Al, which causes the coating to dissolve in the steel, leaving a ferrite phase at the surface with a high Al-content and an excellent high temperature corrosion resistance.

With the coating requirements as a major motive, a specific combination of Cr and Mo has been found to give the best results according to the present invention.

More preferably the steel composition, for a 600 MPa strength combined with a yield ratio lower than 0.65, is defined by the following contents:
- C-content: between 0.095 and 0.125%.

The C-content is determined by the desired strength level.
- Mn-content: between 1.35 and 1.50%. The Mn-content is a cheap alloying element that increases the quenchability. Its level is limited to ensure a sufficient metal coating adhesion for unexposed and exposed automobile parts. The Mn-content also plays an effective role in the interdiffusion of Fe and Al, in the case of an Al-coating.
- Si-content: between 0.10 and 0.15%.

The Si-content is essentially important for hardness and for the flash butt weldability, but has to be limited to ensure sufficient coating adhesion and surface quality.
- Cr-content: higher than 0.2% (for quenchability and for obtaining interdiffusion, in the case of Al-coating) and lower than 0.5% (coating adhesion). The Cr-content is essentially important for quenchability and has to be strictly regulated to assure a sufficient coating adhesion. The effect of a higher Cr-content on the formation of Cr-oxides on the steel sheet surface after soaking and prior to dipping is illustrated in Figure 2. Also, table I describes the growing occurrence of bare spots on the galvanised surface with increasing Cr-and/or Mn content. The appearance of bare spots is an indication of deteriorating metal coating adhesion.
- Mo-content: between 0.1 and 0.25 %, while the relation with the Cr-content is defined by : Cr + 2Mo ≥ 0.7%. The Mo-content is essentially important for quenchability and allows limiting the Cr and Mn contents to an acceptable level assuring a sufficient coating adhesion in the case of hot dip metal coated steel.

The process is preferably characterised by the following steps:

### Hot rolling mill

- T1 : slab-reheating temperature : above 1100°C
- T2 : finishing temperature : 870°C
- T3 : coiling temperature : between 640°C and 670°C

### Cold rolling mill

- Cold rolling reduction comprised between 55% and 63%

After this, there is a difference between the two embodiments of the invention, namely the galvanised steel and the aluminised steel.

In the case of galvanised steel, the next step is :

### Hot dip zinc coating line

- Soaking temperature : 810°C
- Dew point in the hot dip coating line lower than -20°C at the temperatures above 650°C and in the primary cooling stage.
- Primary cooling rate > 40 °C/sec
- Strip temperature at the entry of the molten metal bath: between 460 and 475°C
- Mean secondary cooling rate > 4 °C/s
- Skin-pass reduction: 0.2 %
- Stretch leveller reduction 0 %

### Hot dip aluminising line

- Soaking temperature : 810°C
- Dew point in the hot dip coating line lower than -20°C at the temperatures above 650°C and in the primary cooling stage.
- Primary cooling rate > 40°C/sec
- Strip temperature at the entry of the molten metal bath: between 670°C and 680°C
- Mean secondary cooling rate > 4°C/sec
- Skin-pass reduction : 0%
- Stretch leveller reduction : 0%

The obtained industrial results are represented in Figures 3 and 4 and Table II for galvanised steel and in Table III for aluminised steel.

Figures 5 to 8 represent laboratory results for the aluminised steel according to the invention. Figure 5 illustrates the temperature resistance of the present steel, by way of its weight increase as a function of temperature. The reference 'High Ti ULC steel' refers to a commercially available Al-coated steel with a temperature resistance up to 800 °C. The weight increase of the new steel is significantly lower at 900 °C, which is a consequence of the interdiffusion of Al and Fe, avoiding the formation of a brittle Fe-Al-Si layer and direct oxidation of the steel sheet.

Figure 6 illustrates the conservation and even the slight rise in the mechanical properties (Re and Rm) of the aluminised steel as a function of the number of hours spent at a temperature of 900°C.

Figure 7 illustrates the superior surface quality of the aluminised steel according to the present invention (no flaking at the surface (a) nor cracks in the coating layer (b)).

Figure 8 illustrates the ability of the aluminised steel according to the invention to undergo a reconditioning during cooling, after an exposure to the high temperature. This phenomenon allows to retain the good mechanical properties of the steel, after repeated use at high temperature.

**Table I :**

| Influence of steel composition on the amount of bare spots (#/cm²) detected after galvanising, using the thermal cycle as described within this document | | | | | |
|---|---|---|---|---|---|
| **Cast N°** | **Cr** | **Mn** | **Si** | **Mo** | **Bare spots #/cm**^{**2**} |
| 1 | 0 | 1.54 | 0.12 | 0 | None |
| 2 | 0.25 | 1.44 | 0.12 | 0.2 | None |
| 3 | 0.25 | 1.47 | 0.12 | 0.2 | None |
| 4 | 0.26 | 1.39 | 0.12 | 0.2 | None |
| 5 | 0.5 | 1.5 | 0.08 | 0 | None |
| *6* | *0.7* | *1.5* | *0* | *0* | *> 20* |
| *7* | *0* | *1.9* | *0* | *0* | > *10* |

**Table II :**

| Obtained industrial results of the galvanised steel product according to the present invention. | | | | | | | |
|---|---|---|---|---|---|---|---|
| **Sample N°** | **Skin-pass (%)** | **R**_{**e**} **(MPa)** | **R**_{**m**} **(MPa)** | **A**_{**80**} **(%)** | **n**_{**10-UE**} | **YPE (%)** | **R**_{**e**}**/R**_{**m**} |
| 1 | 0.69 | 375 | 573 | 26 | 0.176 | 0 | 0.65 |
| 2 | 0.71 | 370 | 573 | 26 | 0.178 | 0 | 0.65 |
| 3 | 0.48 | 382 | 592 | 24 | 0.159 | 0 | 0.64 |
| 4 | 0.33 | 363 | 571 | 22 | 0.162 | 0 | 0.64 |
| 5 | 0.2 | 351 | 595 | 26 | 0.168 | 0 | 0.59 |
| 6 | 0.2 | 352 | 590 | 24 | 0.168 | 0 | 0.60 |

**Table III :**

| Mechanical properties of the aluminised steel according to the present invention. | | | | | | | |
|---|---|---|---|---|---|---|---|
| | **R**_{**m**} **(MPa)** | **R**_{**e0,2**} **(MPa)** | **R**_{**e**}**/R**_{**m**} | **A**_{**80**} **(%)** | **A**_{**u**} **(%)** | **n**_{**10-UE**} | **YPE (%)** |
| **Transverse** | 614 | 285 | 0.46 | 20 | 15 | 0.209 | 0 |
| **Longitudinal** | 608 | 280 | 0.46 | 21 | 15 | 0.206 | 0 |

## Claims

1. A steel composition, comprising :
- a C- content between 0.06% and 0.15%,
- a Si-content between 0.1% and 0.4%,
- a Mn-content, lower than 1.5%,
- a Cr-content between 0.2% and 0.5%,
- a Mo-content between 0.1% and 0.25%, so that the following condition is met: Cr + 2Mo ≥ 0.7%,
- the balance being Fe and incidental impurities.

2. The steel composition according to claim 1, wherein the Mn-content is between 1.35% and 1.50%.

3. The steel composition according to claim 1, wherein the Cr-content is between 0.2% and 0.4% and the Mo-content is between 0.15% and 0.25%, so that Cr + 2Mo ≥ 0.7%.

4. The steel composition according to claim 1, wherein the Cr-content is between 0.2% and 0.3% and the Mo-content is between 0.2% and 0.25%, so that Cr + 2Mo ≥ 0.7%.

5. The steel composition according to claim 1, wherein the Si-content is between 0.1% and 0.15%.

6. A method of producing a cold-rolled, metal coated, multi-phase steel, comprising the following steps:
- preparing a steel slab having a composition containing:
- a C-content between 0.06% and 0.15%,
- a Si-content between 0.1% and 0.4%,
- a Mn-content lower than 1.5%,
- a Cr-content between 0.2% and 0.5%,
- a Mo-content between 0.1% and 0.25%, so that the following condition is met: Cr + 2Mo ≥ 0.7%.
- the balance being Fe and incidental impurities,
- preparing a steel sheet by slab re-heating, hot-rolling and cold-rolling,
- soaking said cold-rolled steel sheet at a temperature comprised between Ac1 and Ac3,
- performing a primary cooling down to the temperature of the molten metal bath, with a cooling rate, higher than 25°C per second,
- performing the hot dip metal coating of said steel sheet,
- performing a secondary cooling of said sheet to a temperature lower than Ms, with a cooling rate, higher than 4°C per second,
- performing a skin-pass reduction between 0% and 0.4%.

7. The method according to claim 6, wherein the cooling rate during the primary cooling step is higher than 40°C per second.

8. The method according to claim 6, wherein the steel sheet is galvanised, the temperature at the entry of the molten zinc bath lying between 440°C and 475°C.

9. The method according to claim 6, wherein the steel sheet is aluminised, the temperature at the entry of the molten aluminium bath lying between 650°C and 720°C.

10. The method according to claim 6, wherein the soaking temperature is comprised between 780°C and 850°C.

11. The method according to claim 6, wherein the steel sheet is galvanised, the skin-pass reduction being 0.2%.

12. A cold-rolled, metal-coated, multiphase product, having a steel composition according to claim 1, said product being **characterised by** a tensile strength of at least 500 MPa, and a yield ratio lower than 0.65 in skinned condition.

13. A cold-rolled, metal coated, multiphase product, having a steel composition according to claim 1,said steel being **characterised by** a tensile strength of at least 500 MPa, and a yield ratio lower than 0.6 in unskinned condition.

14. An aluminised steel product according to claim 12 or 13 having a temperature corrosion resistance up to a temperature of 900°C.

## Patentansprüche

1. Stahlzusammensetzung, die enthält:
• einen C-Gehalt, zwischen 0,06% und 0,15%,
• einen Si-Gehalt, zwischen 0,1% und 0,4%,
• einen Mn-Gehalt, kleiner als 1,5%,
• einen Cr-Gehalt, zwischen 0,2% und 0,5%,
• einen Mo-Gehalt, zwischen 0,1% und 0,25%, so dass die folgende Bedingung erfüllt ist: Cr + 2Mo 0,7%,
• wobei der Rest aus Fe und aus zufälligen Verunreinigungen besteht.

2. Stahlzusammensetzung gemäss Anspruch 1, wobei der Mn-Gehalt zwischen 1,35% und 1,50% liegt.

3. Stahlzusammensetzung gemäss Anspruch 1, wobei der Cr-Gehalt zwischen 0,2% und 0,4% liegt und der Mo-Gehalt zwischen 0,15% und 0,25% liegt, so dass Cr + 2Mo 0,7%.

4. Stahlzusammensetzung gemäss Anspruch 1, wobei der Cr-Gehalt zwischen 0,2% und 0,3% liegt und der Mo-Gehalt zwischen 0,2% und 0,25% liegt, so dass Cr + 2Mo 0,7%.

5. Stahlzusammensetzung gemäss Anspruch 1, wobei der Si-Gehalt zwischen 0,1% und 0,15% liegt.

6. Verfahren für die Herstellung eines kaltgewalzten, metallbeschichteten Mehrphasenstahls, das folgende Schritte umfasst:
- die Herstellung einer Bramme aus Stahl mit einer Zusammensetzung, die enthält:
• einen C-Gehalt, zwischen 0,06% und 0,15%,
• einen Si-Gehalt, zwischen 0,1% und 0,4%,
• einen Mn-Gehalt, kleiner als 1,5%,
• einen Cr-Gehalt, zwischen 0,2% und 0,5%,
• einen Mo-Gehalt, zwischen 0,1% und 0,25%, so dass die folgende Bedingung erfüllt ist: Cr + 2Mo 0,7%,
• wobei der Rest aus Fe und aus zufälligen Verunreinigungen besteht,
- die Herstellung eines Stahlbleches durch Wiedererwärmen, Warmwalzen und Kaltwalzen der Bramme,
- das Halten des besagten kaltgewalzten Stahlbleches während einer längeren Zeit auf einer zwischen Ac1 und Ac3 liegenden Temperatur,
- das Durchführen einer primären Abkühlung herunter auf die Temperatur des geschmolzenen Metallbades, mit einer Abkühlungsgeschwindigkeit, die höher als 25°C pro Sekunde ist,
- das Durchführen der Schmelztauchbeschichtung des besagten Stahlbleches mit Metall,
- das Durchführen einer sekundären Abkühlung des besagten Bleches herunter auf eine Temperatur, die kleiner als Ms ist, mit einer Abkühlungsgeschwindigkeit, die höher als 4°C pro Sekunde ist,
- das Durchführen eines Dressiergrades, der zwischen 0% und 0,4% liegt.

7. Verfahren gemäss Anspruch 6, wobei die Abkühlungsgeschwindigkeit während des primären Abkühlungsschrittes höher als 40°C pro Sekunde ist.

8. Verfahren gemäss Anspruch 6, bei welchem das Stahlblech verzinkt wird, wobei die Temperatur am Eingang des geschmolzenen Zinkbades zwischen 440°C und 475°C liegt.

9. Verfahren gemäss Anspruch 6, bei welchem das Stahlblech aluminiert wird, wobei die Temperatur am Eingang des geschmolzenen Aluminiumbades zwischen 650°C und 720°C liegt.

10. Verfahren gemäss Anspruch 6, wobei die Warmhaltetemperatur zwischen 780°C und 850°C liegt.

11. Verfahren gemäss Anspruch 6, bei welchem das Stahlblech verzinkt wird, wobei der Dressiergrad 0,2% beträgt.

12. Kaltgewalztes, metallbeschichtetes Mehrphasenprodukt mit einer Stahlzusammensetzung gemäss Anspruch 1, wobei das besagte Produkt durch eine Zugfestigkeit von mindestens 500 MPa und ein Streckgrenzenverhältnis von weniger als 0,65 im dressierten Zustand gekennzeichnet ist.

13. Kaltgewalztes, metallbeschichtetes Mehrphasenprodukt mit einer Stahlzusammensetzung gemäss Anspruch 1, wobei der besagte Stahl durch eine Zugfestigkeit von mindestens 500 MPa und ein Streckgrenzenverhältnis von weniger als 0,6 im nicht dressierten Zustand gekennzeichnet ist.

14. Aluminiertes Stahlprodukt gemäss Anspruch 12 oder 13 mit einer Korrosionsfestigkeit bis zu einer Temperatur von 900°C.

## Revendications

1. Composition d'acier comprenant :
- une teneur en C entre 0,06% et 0,15%,
- une teneur en Si entre 0,1% et 0,4%,
- une teneur en Mn inférieure à 1,5%,
- une teneur en Cr entre 0,2% et 0,5%,
- une teneur en Mo entre 0,1% et 0,25%, de sorte que la condition suivante soit remplie : Cr + 2Mo ≥ 0,7%,
- le restant étant formé de Fe et d'impuretés fortuites.

2. Composition d'acier selon la revendication 1, dans laquelle la teneur en Mn se situe entre 1,35% et 1,50%.

3. Composition d'acier selon la revendication 1, dans laquelle la teneur en Cr se situe entre 0,2% et 0,4% et la teneur en Mo se situe entre 0,15% et 0,25%, de sorte que Cr + 2Mo ≥ 0,7%.

4. Composition d'acier selon la revendication 1, dans laquelle la teneur en Cr se situe entre 0,2% et 0,3% et la teneur en Mo se situe entre 0,2% et 0,25%, de sorte que Cr + 2Mo ≥ 0,7%.

5. Composition d'acier selon la revendication 1, dans laquelle la teneur en Si se situe entre 0,1% et 0,15%.

6. Procédé de production d'un acier multiphase, revêtu de métal, laminé à froid, comprenant les étapes suivantes :
- préparation d'une brame d'acier ayant une composition contenant :
- une teneur en C entre 0,06% et 0,15%,
- une teneur en Si entre 0,1% et 0,4%,
- une teneur en Mn inférieure à 1,5%,
- une teneur en Cr entre 0,2% et 0,5%,
- une teneur en Mo entre 0,1% et 0,25%, de sorte que la condition suivante soit remplie : Cr + 2Mo ≥ 0,7%,
- le restant étant formé de Fe et d'impuretés fortuites,
- préparation d'une tôle d'acier par re-chauffage, laminage à chaud et laminage à froid de la brame,
- maintien de ladite tôle d'acier laminée à froid à une température comprise entre Ac1 et Ac3,
- refroidissement primaire à la température du bain de métal fondu à une vitesse de refroidissement supérieure à 25°C par seconde,
- revêtement métallique à chaud de ladite tôle d'acier,
- refroidissement secondaire de ladite tôle à une température inférieure à Ms à une vitesse de refroidissement supérieure à 4°C par seconde, et
- réduction du skin-pass entre 0% et 0,4%.

7. Procédé selon la revendication 6, dans lequel la vitesse de refroidissement au cours de l'étape de refroidissement primaire est supérieure à 40°C par seconde.

8. Procédé selon la revendication 6, dans lequel la tôle d'acier est galvanisée, la température à l'entrée du bain de zinc fondu se situant entre 440°C et 475°C.

9. Procédé selon la revendication 6, dans lequel la tôle d'acier est aluminisée, la température à l'entrée du bain d'aluminium fondu se situant entre 650°C et 720°C.

10. Procédé selon la revendication 6, dans lequel la température de maintien est comprise entre 780°C et 850°C.

11. Procédé selon la revendication 6, dans lequel la tôle d'acier est galvanisée, la réduction du skin-pass étant de 0,2%.

12. Produit multiphase, revêtu de métal, laminé à froid, ayant une composition d'acier selon la revendication 1, ledit produit étant **caractérisé par** une résistance à la traction d'au moins 500 MPa et un rapport d'élasticité inférieur à 0,65 avec skin-pass.

13. Produit multiphase, revêtu de métal, laminé à froid, ayant une composition d'acier selon la revendication 1, ledit acier étant **caractérisé par** une résistance à la traction d'au moins 500 MPa et un rapport d'élasticité inférieur à 0,6 sans skin-pass.

14. Produit d'acier aluminisé selon la revendication 12 ou 13, ayant une résistance à la corrosion jusqu'à une température de 900°C.
